

July 16, 1929.

H. E. COLEY

1,721,373

PROCESS FOR THE MANUFACTURE OF ZINC

Filed Aug. 8, 1927.



Inventor  
Henry E. Coley

By

J. Kaplan  
attorney

## UNITED STATES PATENT OFFICE.

HENRY EDWIN COLEY, OF LONDON, ENGLAND.

## PROCESS FOR THE MANUFACTURE OF ZINC.

Application filed August 8, 1927, Serial No. 211,293, and in Great Britain February 2, 1927.

This invention relates to a process of manufacturing zinc wherein a hydrocarbon or hydrocarbon containing body is employed the hydrocarbon being decomposed to form 5 a reducing agent to effect the reduction of the ore, oxide or the like. In this respect the process according to the present invention is similar to other processes in which a solid, liquid, or gaseous hydrocarbon is 10 used as an aid to reduction. But whereas in all known processes of this character carbon in the ordinary or molecular state is formed and effects the reduction, by the present process carbon in statu mescendi or 15 in the atomic state is produced and in this state is caused to react on the ore to be reduced. This has the effect of reducing the ore more rapidly and more completely than is possible by carbon in the ordinary or 20 molecular state.

I have found that to produce and use the carbon in its nascent or atomic state the heat necessary for effecting its decomposition must be imparted to it by, and as a result of, 25 actual contact with the ore to be reduced and such ore, as a consequence, must first of all have been brought up to a temperature which is sufficient to enable the reduction to take place and to both effect the decomposition of the hydrocarbon at the moment of its first contact and to continue to effect the decomposition of the continuing supply of hydrocarbon.

The essential feature of the process according to the present invention being the utilization of carbon in its nascent or atomic state for effecting the reduction it follows that the carbon in this state can be obtained 35 from a hydrocarbon which is initially in a solid, liquid, or gaseous form or from a body containing or forming a hydrocarbon the only essential being that such hydrocarbon is not allowed to decompose before 40 it has actually come into contact with ore previously heated to a reducing temperature.

For a proper understanding to be obtained of the different sets of conditions which occur in producing on the one hand carbon in the ordinary or molecular state 45 and on the other hand carbon in the nascent or atomic state it must be realized that unless the hydrocarbon is allowed to attain its

critical or decomposition temperature only at the moment of its contact with the ore to be reduced and by reason of this contact 55 carbon in its ordinary or molecular state is always formed. On the other hand by allowing the hydrocarbon to be brought to its critical or decomposition temperature only at the moment of its contact with the ore 60 and by reason of this contact, carbon in a nascent or atomic state is always released and never in its ordinary or molecular state.

By experiments I have found the following to be facts:—

65

(1) If the hydrocarbon is mixed with the ore and both are simultaneously heated up to the reducing temperature of the ore, carbon in the ordinary or molecular state will be released. This occurs repeatedly 70 without exception as decomposition of the hydrocarbon always takes place before the ore has attained its reducing temperature.

(2) If the ore is heated up to the reducing temperature first and a hydrocarbon is 75 projected into the heated reducing chamber above the ore decomposition of the hydrocarbon takes place before the hydrocarbon can possibly reach the ore and carbon in the ordinary or molecular state is released. 80 This is proved by the fact that soot is deposited over the surface of the ore.

(3) If a large quantity of a cold hydrocarbon gas is rapidly blown through the heated ore within the reducing chamber the 85 ore is thereby cooled to below its reducing temperature and practically no reduction will take place. By this method it has been found impossible to maintain the ore or the required reducing temperature which for 90 zinc is at or almost 930° centigrade. As a consequence the decomposition of the hydrocarbon takes place when the ore is at a temperature below that necessary for its reduction.

95

(4) If the hydrocarbon is admitted together with air, a flame is produced and as a result the hydrocarbon is obviously thereby decomposed before it can possibly come into contact with the ore. Any reduction 100 which may take place with this method is effected by means of the released hydrocarbon and the CO formed and not by the carbon per se.

As a result of these and other experiments it has been found to be absolutely essential for the ore to be first heated to its reducing temperature and for such heated ore itself to bring the hydrocarbon to its critical or decomposition temperature for carbon to be released in its nascent or atomic state. In this latter state the carbon is in its most active condition and will effect the reduction of the ore far more rapidly and completely than is possible when the carbon is in its ordinary or molecular state.

In practice the premature decomposition of the hydrocarbon is prevented by artificially cooling the pipe or other means used for conveying the hydrocarbon to the ore such as by surrounding the same with a jacket through which water is continuously circulated.

The process of manufacturing zinc according to the present invention consists broadly in heating the ore to be reduced to a suitable reducing temperature and when the ore is at this temperature conveying a hydrocarbon to the ore by means of an artificially cooled conveying means so that the hydrocarbon in its non-decomposed condition reaches the ore and as a result of actual contact with the ore is decomposed and produces carbon in a nascent state.

A hydrocarbon such as crude oil, petroleum or the like or a suitable body containing hydrocarbon such as coal, peat, lignite and the like may be used to effect a reduction by the process forming the present invention.

The relative quantities of ores or the like to hydrocarbon used depend upon two factors viz.—the zinc content of the material and the nature of the hydrocarbon used and may be best described by the following equation:—



In this equation the hydrocarbon represented by the formula  $\text{C}_6\text{H}_{14}$  is given as being typical only.

In the application of my invention it is necessary to carry out the reaction in an apparatus of suitable construction, so designed that while the process is being carried out air may be excluded if desired from the apparatus and preferably designed that the material to be treated may be passed continuously through the apparatus. The apparatus may be made of any suitable material but this material depends upon the nature of the ore or oxide to be treated and upon the temperature at which the reaction must take place. The apparatus may consist of a chamber or cylinder which can be rotated in order to provide agitation to the ores, etcetera to be treated, or which may be fixed and provided with internal agitating means such as rotary baffles, so that the

material is subjected to frequent agitation during its passage through the apparatus.

A suitable apparatus for carrying into effect a process according to the present invention is illustrated in the accompanying drawings which apparatus is designed particularly for the manufacture of zinc and like volatile metals.

In the drawings:—

Fig. 1 is a longitudinal elevation, partly in section, of the apparatus.

Fig. 2 is a similar view taken at right angles to Fig. 1 and illustrating the means for preheating the ore and feeding the same to the main tube.

The apparatus illustrated in the drawings comprises a rotatable tube 1 constituting the reducing chamber. This tube which is adapted to be heated preferably externally and entirely or partly by the burning of the gas produced by the reaction is supported upon rollers which engage circumferential flanges 3 on the exterior of the tube. These rollers are preferably of a comparatively large diameter and either the rollers or the flanges 90 may be of increasing width towards one end of the tube to allow for the expansion of the tube.

The tube although sealed to prevent the free ingress of air is so constructed and arranged as to allow for the introduction of the ores or the like at one end and the extraction of the gangue at the other end. The reduced metal passes out with and at the same end of the tube as the gases.

The hydrocarbon or hydrocarbon containing body when in the liquid form may be led into the interior of the tube at either end by way of a water cooled pipe 4 which as indicated by the dotted lines extends down the interior of the tube a distance suitable for the effective working of the process. If the hydrocarbon or hydrocarbon containing body is not in the liquid form it may be led into the interior of the tube by means of a water cooled or other artificially cooled conveyor. By this means the hydrocarbon is caused to maintain its original or non-decomposed condition until the same actually comes into contact with the heated ore or the like within the tube 1 when the hydrocarbon undergoes decomposition, yielding products of a highly active reducing nature such as nascent carbon, nascent hydrogen etcetera.

This pipe 4 is surrounded by an outer jacket 5 through which in the present example a stream of water is caused to circulate.

The inlet for such cooling water is indicated at 6 and its outlet at 7. By this means the hydrocarbon is caused to maintain its original condition until the same actually comes into contact with the heated ore or the like within the tube 1 when it disinte-

grates and forms nascent carbon which effects the reduction of the ore or the like to its metal.

The ore or the like before being introduced into the tube 1 is preheated to preferably a reducing temperature. This is effected in the example illustrated by passing the same through a rotating tube 8, see Fig. 2, which is disposed at right angles to the main tube 1. The preheated tube 8 is fed from a hopper 9 by means of a suitable conveyor 10 and it discharges the preheated ore into the feed hopper 11 of the main tube 1.

15 From this hopper 11 the ore is conveyed, by means of the conveyor 12, through the wall of and into the interior of a casing forming one part of the gas take-off or vapour outlet 13. From the interior of this 20 casing the ore is picked up by means of a scoop 14, mounted upon one end of and revolving with the main tube 1 which is set at a slight declination so that the ore works its way slowly through the tube to the opposite end.

As before described the hydrocarbon containing body may be introduced at the opposite end of the tube to that into which the fresh ore is introduced. As a consequence 30 of this fact and the fact that the ore is preheated to at or about a reducing temperature before it is passed into the reducing tube a reducing process goes on throughout practically the entire length of the reducing tube. By this means the complete reduction desired is facilitated in that the reducing agent when in a condition of least 35 activity comes into contact with the fresh and therefore richest ore at the inlet end 40 of the tube whilst the poorest ore which is not affected by the reducing agent in this condition is subjected to the hydrocarbon at or adjacent to the point of its introduction into the reducing tube.

45 The reduced metal in the form of a vapour passes out of the tube 1 with the gases through the vapour outlet 13 whilst the gangue is discharged into the receptacle 15 from the bottom of which it is continuously removed by means of the conveyor 16.

It will thus be seen that by means of an apparatus as above described the process is a continuous one, the cold ore being fed into the hopper 9 and the gangue discharged 50 automatically and continuously by the conveyor 16.

Air is excluded from the tube during the process to prevent re-oxidation of the metal and this is effected by the provision of gas tight joints at both ends of the tube.

Owing to the temperature at which the joint at the gas take-off end of the tube is required to work, existing types of joint are unsuitable.

65 The joint at this end, according to the

example illustrated comprises a stationary outer casing 17 forming part of or attached to the inner end of the casting forming the gas take-off 13. This casing consists of an annular plate 18, and a circumferential flange 19 extending horizontally from the plate and disposed concentric with the aperture in the plate. The plate 18 is bolted or otherwise secured to the gas take-off casting 13. The corresponding end of the tube 1 is formed with a circumferential flange 20 disposed a short distance in from the end of the tube.

When the apparatus is assembled the gas take-off end of the tube 1 projects through the aperture in the plate 18 and the flange 20 on this end of the tube resides within the shrouding formed by the horizontal flange 19. The required gas tight joint is formed by interposing a suitable packing 21 between the opposing faces of the flange 20 on the tube and the plate 18 and applying spring or other pressure to the tube 1 so as to hold the flange 20 hard against the packing and to compensate for expansion of the tube 1.

From experiments so far made I have found that the most suitable packing is a machined block of wrought iron. Such a packing material besides providing a gas tight joint will stand up to the high temperature to which it is normally subjected. Any other suitable metal or alloy of metals may however be used in lieu of the wrought iron.

From my experiments in this direction I have found that iron or steel wire, preferably in rope form, constitutes a suitable packing material which besides providing a gas tight joint stands up to the high temperatures to which it is normally subjected.

The above mentioned pressure is applied in the example illustrated through the medium of a bell crank lever 22, a spring 23 or springs acting upon one arm of such lever, the other arm applying pressure to a suitable surface 24 on the tube through a roller 23 or other anti-friction device. The pressure thus acts in a direction axial of the tube.

The gangue discharge end of the tube may be supported in any suitable manner so as to exclude air but preferably by means of a bearing having a stuffing box 26 and a gland packing 27.

#### Claims:

1. A method of reducing zinc-bearing material which consists in agitating in an air excluding tube a mass of said material heated to substantially its reduction temperature, and when at that temperature introducing a hydrocarbon cooled below its decomposition temperature into said tube at a point below the upper surface of said mass.

2. A method of reducing inc-bearing material which consists in heating a mass of said material to substantially its reduction

temperature, agitating the same in an air excluding vessel and when at that temperature introducing a hydrocarbon cooled below said temperature at a point normally covered by said mass.

3. A method of reducing zinc-bearing material which consists in heating a mass of said material to substantially its reduction temperature within a vessel, conducting a

hydrocarbon within the said vessel, cooling <sup>10</sup> the hydrocarbon below its decomposition temperature during its passage into the vessel and up to the moment of contact with the heated mass of material, and then contacting the cooled hydrocarbon with the mass of <sup>15</sup> material heated to its reduction temperature.

In testimony whereof I affix my signature.

HENRY EDWIN COLEY.